

# UNITED STATES PATENT OFFICE.

CARLETON ELLIS, OF MONTCLAIR, NEW JERSEY, ASSIGNOR TO NEW JERSEY TESTING LABORATORIES, A CORPORATION OF NEW JERSEY.

## PROCESS OF TREATING MASSES OF CONCRETE.

1,130,717.

Specification of Letters Patent.

Patented Mar. 9, 1915.

No Drawing.

Application filed September 25, 1911. Serial No. 651,185.

To all whom it may concern:

Be it known that I, CARLETON ELLIS, a citizen of the United States, and a resident of Montclair, in the county of Essex and State of New Jersey, have invented certain new and useful Processes of Treating Masses of Concrete, of which the following is a specification.

This invention relates to a method of treating cement or concrete surfaces and relates in particular to the treatment of concrete floor structures and the like, to form a mass of concrete substantially free from rapid abrasion and dusting.

Concrete would be an ideal material for flooring purposes if it were not prone to abrade under the attritive action caused by walking thereover. In office and public buildings, mills and shops, the dust so produced is an especial nuisance and many efforts have been made to overcome the difficulty, but without satisfactory results.

The usual method is to flood the surface with a hard varnish so that a film of the dried varnish surfaces the concrete. Owing to the lack of resiliency of concrete such a surface even if secured by the use of several coats of very hard drying varnish, is easily abraded. Water glass, fluosilicates, and various drying oils have been used without satisfactory elimination of dusting.

Floor concrete usually is given a troweled surface or granolithic effect and the finishing coat is generally of high cement and low sand content. Also by troweling the finer particles of cement and sand work toward the surface while the coarser particles sink beneath. This results in a glazed or smooth surface to which varnish coatings do not cling readily and the density of the extreme surface layer prevents penetration of the varnish to any great extent. Such coatings readily peel and repainting or recoating is soon required.

In the present invention the surface of the concrete mass is left open to secure proper penetration of the coating or as this is often impracticable the troweled or granolithic finish is etched with acid and the like after setting or washed with water just after the initial set and before the final set, or in other ways roughened so that the surface of nearly neat cement is evenly etched or opened so as to permit of the subsequent treatment. After drying such an opened

surface the coating material is plied. The first coat should be rather thin in body, preferably, so as to secure a substantial anchoring foothold. Subsequently one or more coats of the material are applied to build up a stratum in and around the particles of concrete or cement which has a mean height substantially that of the average height of the projecting granules or rugosities of the roughened surface. Thus several important advantages are secured by this procedure. First, the coating is securely anchored to the surface; second, the peaks or uppermost points of the rugosities form a frictional foothold, which overcomes the slippery character of some varnish coatings; third, the aforesaid peaks projecting more or less from their bedding divert wear from the coating itself; fourth, the surface may be waterproofed in a more satisfactory way than by coatings which are simply on the surface and having poor adherence thereto; fifth, moisture and heat do not have a tendency to cause blistering; sixth, dusting may be effectually prevented.

In carrying out my invention I preferably as stated roughen the surface of the concrete mass with acid, using for example a five or ten per cent. solution of hydrochloric acid, or a fifteen per cent. solution of sodium bisulfate, or similar acid wash. A mixture of three parts of sodium bisulfate to one part of magnesium chlorid is useful, as roughening is secured without material weakening of the bonding of the set cement. This mixture is used in about the proportion of one and one half pounds to the gallon of water. These roughening washes are allowed to remain on the surface until the desired degree of rugosity is secured, when the surface is washed and dried. The surface is now ready to be treated with the coating or impregnating waterproofing or hardening material. The selection of the material for this purpose depends to some extent on the service to which it is to be put. For office buildings and the like of a generally dry character a short oil varnish may be used. This may be prepared from copal gum, such as Manila, kauri, Zanzibar, Pontianak, Borneo and the like, with wood oil or other drying oil capable of producing a tough film with varnish gum after suitable heat treatment, or Pontianak rubber resin may be used with a drying oil, with or with-

- out additions of the resins mentioned. As Pontianak rubber resin is substantially unsaponifiable it is well adapted for such uses, as it is not affected by cement alkali. However under the present invention there is no longer need of using expensive hard gums and oils for surface treatment, as the rugosities of the surface protect the waterproofing film from material abrasion for a long time.
- 10 Much cheaper materials, such as solutions of Pontianak rubber resin or Manila resin and the like in a hydrocarbon solvent may be used, and although more brittle than the oil varnishes they are sufficiently protected by the rugosities so that they are preserved from abrasion for an indefinite time. A small amount of ceresin or paraffin wax or other waxy body gives a slight tempering effect without materially affecting the cost.
- 15 Larger amounts soften the resins considerably and in such cases the rugosities are made quite prominent, so that the softer material is better protected. Tetrachlornaphthalene and also pentachlornaphthalene are extremely good waterproofing agents and when mixed with resins in about equal proportions and suitably thinned form a dust preventing and waterproofing material which is excellent for mill floors and factories where dampness prevails, or where acids or other chemical reagents are employed.
- 20 As stated, the first coat should preferably be of thin consistency so as to secure effective penetration and form an anchoring layer. Subsequent coats are better applied of heavier body so as to quickly fill the depressions to practically the level of the surface peaks, or thereabout. Various pigments may be used in the floor coatings as well as the usual filling and extending materials. The addition of rather coarsely ground silex, pumice and the like secures greater frictional foothold. Pulverized alundum is especially satisfactory in this respect, as a small quantity serves for a large surface and the attritional or frictional reinforcement to the peaks of natural origin obtained in this way is extremely useful in floors subjected to extreme service conditions. Carborundum also may be used, although this material has certain disadvantages which do not appear with alundum and similar artificial peak-formers.
- 25 Instead of using surface filling materials of a varnish character, other compositions may be used, as for example, a mixture of zinc oxid and zinc chlorid, or of magnesium oxid and chlorid, preferably admixed with artificial peak-forming material of an extremely hard nature. For example the surface may be treated with zinc oxid and alundum in water which has been bodied with a little alkali-casein and after drying a concentrated solution of zinc chlorid is applied.

A zinc oxychlorid cement forms and as soon as this has set the surface may be washed and dried. If desired a coating of varnish may be applied over this.

The condensation products of carbolic acid other cresol or other phenol may some time be employed to good advantage, especially when the cement is naturally rough and open and has not been etched with acid. Condensation products made with either an acid or alkaline condensing or catalytic agent may be employed and if desired the surface, after coating or impregnation, may be heated to superficially form a hard, infusible, condensation product of great durability.

If the cement flooring or its upper layers carry a waterproofing agent of the integral type, such as magnesium or calcium stearate or resinate, the dust-preventing coating need not be of as waterproof a character as when ordinary cement-concrete is to be treated. Nitrocellulose solutions may be used in such cases.

Having described my invention, to the details of which description I do not wish to be limited, what I claim is:—

1. The process of treating masses of concrete which comprises roughening a surface thereof in impregnating such surface with a water-resistant binding material and in filling the depressions of said surface substantially to a level with the peaks thereof, with a dust-preventing and waterproofing material; whereby the wear is taken substantially by said peaks.

2. The process of treating masses of concrete which comprises roughening a surface thereof in impregnating such surface with a water-resistant binding material and in filling the depressions of said surface substantially to a level with the peaks thereof, with a dust-preventing and waterproofing material of a finish coating character; whereby the wear is taken substantially by said peaks.

3. The process of treating masses of concrete which comprises roughening a surface thereof in impregnating such surface with a water-resistant material as an anchoring coat or layer and in filling the depressions of said surface substantially to a level with peaks thereof, with a material of a dust-preventing and waterproofing character, carrying an extremely hard granular abrasive serving as frictional material; whereby the wear is taken substantially by said peaks.

4. The process of treating masses of concrete and similar material used for flooring purposes which comprises roughening the surface thereof by removal of very fine cement material and consequent exposure of coarser aggregate and sand grains, in superficially impregnating the roughened surface

thereof with a water-resistant material as an anchoring layer, and in filling the depressions of said surface substantially to a level with the rugosities thereof, but no 5 higher, with a dust preventing and waterproofing binding material of an organic character; whereby the wear is taken substantially by said peaks.

5. The process of treating masses of concrete which comprises roughening and superficially impregnating a surface thereof with a water-resistant binding material and in filling the depressions of said surface substantially to a level with the peaks thereof, 10 with a dust preventing and waterproofing material of a finish coating character; whereby the wear is taken substantially by said peaks.

6. The process of treating masses of concrete which comprises roughening and superficially impregnating a surface thereof with a water-resistant binding material and in filling the depressions of said surface substantially to a level with the peaks thereof, with a dust preventing and waterproofing material of a finish coating character carrying a hard frictional substance; whereby the wear is taken substantially by 15 said peaks.

Signed at Montclair, in the county of 30 Essex and State of New Jersey, this 22nd day of September, A. D. 1911.

CARLETON ELLIS.

Witnesses:

ROBT. M. HENING,  
ELIZABETH M. MARTIN.